

# UNITED STATES PATENT OFFICE.

GEORGE H. WORRALL, OF KIRKWOOD, MISSOURI, ASSIGNOR TO UNITED LEAD COMPANY, OF NEW YORK, N. Y., A CORPORATION OF NEW JERSEY.

## HARD LEAD ALLOY.

1,360,348.

Specification of Letters Patent. Patented Nov. 30, 1920.

No Drawing. Application filed August 25, 1919, Serial No. 319,669. Renewed May 28, 1920. Serial No. 385,085.

To all whom it may concern:

Be it known that I, GEORGE H. WORRALL, United States citizen, residing in Kirkwood, Missouri, have invented the following-described Improvements in Hard Lead Alloys.

I have discovered that, in small amounts, mercury has the property of increasing the hardness of alloys of lead with certain of the lead-hardening metals and that it improves such alloys in other respects and can be used for this purpose with considerable economy in the cost of production.

The class of alloys on which mercury has this effect include in general, those lead base alloys commonly or most practically produced by electrolytic deposition and those wherein the primary hardening effect upon the lead is produced by small percentages of one or more of the alkaline earth metals and also those containing small amounts of sodium, potassium, magnesium or lithium or combinations of these lead-hardening metals with or without other additions. By way of example of the effect of mercury on these and other alloys it may be stated that the addition of .25% mercury to an alloy containing lead 99.5% and calcium .5% increases the hardness equivalent to that of lead containing nearly twice the amount of calcium, other conditions being constant. Calcium is one of those lead-hardening metals most conveniently combined with lead by electrolytic deposition from its fused salt, and it is therefore apparent that the addition of mercury reduces the time of electrolysis, and hence the cost of production of the alloy by approximately half, while the cost of the mercury itself is trifling by comparison. The mercury also improves the resulting alloy for bearing metal and general casting purposes by rendering it more fluid in its fused state.

The same advantages obtain in varying degrees with other lead-base alloys and I have ascertained that even lead alone is also somewhat hardened by a small addition of mercury. The amount of mercury necessary for the purposes of the invention is variable according to the degree of hardness desired and the character of the metal or metals used with or present in the lead as the main hardening agent and no definite percentage can therefore be prescribed for all materials and conditions. The range lies far below the percentages producing the so-

called amalgams, which are not suitable for bearing metal purposes and in actual practice is confined between the limits .1% and .25% of the whole alloy but with some alloys, one per cent. and even higher percentages 60 produce the characteristic improvements above described. The maximum limit for each composition is the point where the mercury ceases to harden the alloy and in general the practical upper limit of usefulness 65 is around 3% according to my present belief.

Additional ingredients may be introduced into or used with the mercury-hardened alloys of this invention for various purposes such as resisting the tendency to dross or 70 controlling the appearance, weight or otherwise. It has been ascertained that aluminum, in very small amounts, tends to prevent the drossing of lead-base alloys and on this account I prefer to use aluminum in my 75 alloys when necessary. When so used it is introduced in amounts approximately .02% of the whole alloy and inasmuch as aluminum does not readily mix with lead it is generally introduced alloyed with a small 80 amount of tin, zinc or magnesium acting as a carrier, or a mixture of one or more of these metals in small amounts aggregating, for non-drossing purposes, approximately 85 .35% of the total alloy.

The process of manufacture according to this invention comprises first combining the lead with the principal hardening metal, as for example, any of the metals above indicated, namely, calcium, strontium, magnesium, sodium, potassium or lithium, with or without barium, and then while molten or remelted adding the requisite small amount of mercury the resulting alloy being then poured into ingots for shipment and sale. 90 When the primary hardening metal is alloyed with the lead electrolytically, the molten lead constitutes the cathode of an electrolytic cell of which the fused salt or salts of the hardening metals, constitute the electrolyte, the anode being the usual carbon electrode of the cell. Electrolysis is continued until a predetermined amount of the hardening metal or metals has been absorbed by the lead whereupon the molten alloy is removed to another vessel and when somewhat cooled the mercury is added in amount sufficient to raise the hardness to the point previously determined upon. The non-drossing agent and such other ingredi- 100 105 110

ents as are desired may also be added at the same time and preferably previously to the addition of the mercury. I prefer at present to use my invention according to the following formula which includes two of the alkaline earth metals as the main hardening agent:—

10 Barium between .90 and 1.10%, calcium between .40 and .60%, mercury between .10 and .25%, to which is added to the extent of about .35%, a mixture of the zinc or magnesium with aluminum and sufficient to carry about .02% of aluminum into the alloy. The balance of the alloy is lead. The 15 barium and calcium are first alloyed with the lead electrolytically as above described, the alloying process being continued for such period as will produce substantially the indicated proportions of these metals and a 20 hardness less than desired in the product alloy. Whereupon, in another vessel, an amount of mercury sufficient to bring the hardness up to the desired point is added together with the non-drossing ingredient. 25 In this manner a predetermined degree of hardness may be obtained with accuracy. The proportions above stated produce a 30 degree of hardness approximating 25 or better on the Brinell scale. The alloy is tough and excellently adapted for all bearing metal purposes and for general die-casting. Certain specific combinations of the 35 metals herein mentioned but not specifically claimed form the subjects of collateral applications.

Claims:

1. The method of making lead alloys of predetermined hardness which consists in hardening a lead base alloy containing upward of 90% lead by adding thereto a small percentage of mercury.
2. The method of making hard lead alloys of predetermined hardness which consists in compounding lead with a lead hardening

metal or metals in amounts adapted to produce a certain degree of hardness and increasing such hardness to a predetermined point by introducing a small percentage of mercury in the composition.

3. The method of making lead base alloys 50 which consists in electrolytically alloying therewith a lead-hardening agent and thereafter increasing the hardness of such alloy by adding thereto a small percentage of mercury.

4. A hard lead alloy suitable for bearings and like uses containing upward of 90% lead, a lead hardening metal and a small percentage of mercury coating therewith to increase the hardness of the alloy.

5. A metallic composition suitable for bearings and like purposes comprising an alloy containing lead 90% or upward, a lead-hardening metal and a small percentage of mercury coating with said metals 65 to increase the hardness thereof.

6. A hard lead alloy containing lead and one or more metals of the alkaline earth metals and having its hardness increased by the presence therein of a small percentage 70 of mercury.

7. An alloy comprising upward of 90% lead, calcium and a small percentage of mercury.

8. An alloy comprising upward of 90% 75 lead, two or more lead-hardening metals and a small percentage of mercury.

9. A hard lead alloy comprising lead, calcium, barium and a small percentage of mercury.

10. A hard lead alloy containing between .9% and 1.10% barium, between .4% and .6% calcium and between .10% and .25% mercury.

In testimony whereof I have signed this 8 specification.

GEORGE H. WORRALL.